

# United States Patent Office

3,809,706

Patented May 7, 1974

1

3,809,706

## N-SUBSTITUTED FATTY ACID AMIDE LUBRICANTS

Frank C. Magne, Robert R. Mod, and Gene Sumrell, New Orleans, La., and Winfred E. Parker, Philadelphia, Pa., assignors to the United States of America as represented by the Secretary of Agriculture

No Drawing. Original application Aug. 31, 1971, Ser. No. 176,734, now Patent No. 3,746,644. Divided and this application Apr. 6, 1973, Ser. No. 348,802

Int. Cl. C07f 9/02, 9/10

U.S. Cl. 260—403

1 Claim

### ABSTRACT OF THE DISCLOSURE

This invention relates to N-acylmorpholines and N-mono and N,N-disubstituted fatty acid amides and to similar derivatives of epithioamides which are useful as base and extreme pressure lubricants and additives.

This is a division of application Ser. No. 176,734 filed Aug. 31, 1971, now Pat. No. 3,746,644.

A non-exclusive, irrevocable, royalty-free license in the invention herein described, throughout the world for all purposes of the United States Government, with the power to grant sublicenses for such purposes, is hereby granted to the Government of the United States of America.

This invention relates to certain compounds which are N-fatty acyl derivatives of primary and secondary amine and N-substituted acyl derivatives of primary and secondary amines which have exhibited utility as base lubricants, extreme pressure lubricants or lube additives. More particularly, this invention relates to N- and N,N-disubstituted long chain aliphatic amides the acyl component of which is a normal, branched, or substituted alkenoic or alkanoic acyl group containing from 16 to 22 carbon atoms the amide nitrogen of which may be derived from an alkyl amine, dialkyl amine, alkylalkoxyalkylamine, dialkoxyalkylamine or nitrogen heteroalicyclic. Typical amines are butylamines, dibutylamines, N-methyl-alkoxyethyl amine, di-ethoxyethyl amine, and morpholine. The acyl substituent referred to may be divalent sulfur or pentavalent phosphorus.

We have discovered that many of the simple N-alkyl and N,N-dialkyl or N-alkyl-N-alkoxyalkyl amides of the C<sub>16</sub> to C<sub>22</sub> alkenoic or alkanoic fatty acids are good base lubricants. We have further discovered that the introduction of divalent sulfur into the fatty acid moiety imparts excellent extreme pressure lubricant characteristics to such compounds. In particular we have found the epithio group



to be most effective. We have also observed that the introduction of both hydroxy and alkyl phosphato groupings alpha to each other also imparts extreme pressure lubricant characteristics to the compound.

In addition it was noted that the above hydroxyphosphato compound and its mercapto analog N-[9(10)-mercapto-(9)10-dibutylphosphato]stearamide were effective antiwear compounds and additives.

Included among the specific compounds operable as base lubricants are N-methyl-N-butyloleamide, N-ethoxyethoxyethoxy propyloleamide, N-ethoxyethoxy propyloleamide, N-methoxyisopropylolamide, N-methoxyethyleamide. Compounds showing particular promise as extreme pressure lubricants or additives are N,N-dibutyl-9, 10-epithiostearamide, N,N-dibutyl-9, 10-12, 13-diepithiostearamide, 9, 10-epithiostearoyl morpholine, N-

2

ethoxyethoxyethoxypropyl-9, 10-epithiostearamide, n-9, 10-12, 13-diepithiostearoylmorpholine and N-[9(10)-hydroxy-9(10)-dibutylphosphato]stearamide.

Compounds showing particular promise as antiwear additives are N,N-dibutyl-[9(10)-hydroxy-(9)10-dibutylphosphato]stearamide and N,N-[9(10)mercapto-(9)10-dibutylphosphatostearoyl]morpholine.

#### Example 1

10 N-methyl-N-butyloleamide.—100 grams (0.33 mole) of oleoyl chloride was added dropwise and with stirring to a mixture of 29 grams (0.33 mole) of N-methyl-N-butyamine and 27 grams (0.33 mole) of pyridine. Stirring was continued until the heat of reaction subsided. 15 The solid pyridine hydrochloride was filtered off and the filtrate was washed successively with aqueous HCl and water until acid free. It was dried stripped, percolated through an activated alumina column, and the product removed from the percolate by stripping off the solvent. 20 Analysis of the product (percent): C, 78.87 (theory 78.63); H, 13.02 (theory 12.82); N, 3.96 (theory 3.99).

#### Example 2

25 N,N-dibutyloleamide.—This material was prepared by the procedure of Example 1 from 100 grams (0.33 mole) of oleoyl chloride 42.5 grams (0.33 mole) of di-n-butyamine and 27 grams (0.33 mole) pyridine. Analysis of the product (percent): C, 78.94 (theory 79.25); H, 13.16 (theory 13.06); N, 3.44 (theory 3.56) confirm the preparation.

#### Example 3

30 Ethoxyethoxyethoxy propyloleamide.—This material was prepared by the procedure of Example 1 from 100 grams (0.33 mole) of oleoyl chloride, 73.0 grams (0.33 mole) ethoxyethoxyethoxy-propylamine and 27.0 grams (0.33 mole) pyridine. Analysis (percent): C, 71.84 (theory 72.04); H, 11.80 (theory 11.80); and N, 2.96 (theory 2.90) confirm the preparation.

#### Example 4

35 Ethoxyethoxypropyloleamide.—This material was prepared by the procedure of Example 1 from 100 grams (0.33 mole) of oleoyl chloride, 58.3 grams (0.33 mole) ethoxyethoxypropylamine and 27.0 grams (0.33 mole) of pyridine. Analysis (percent): C, 71.45 (theory 73.80); H, 11.87 (theory 12.07); and N, 2.92 (theory 3.18) confirm the preparation.

#### Example 5

40 Methoxyisopropylolamide.—This material was prepared by the procedure of Example 1 from 100 grams (0.33 mole) of oleoyl chloride, 29.3 grams (0.33 mole) methoxyisopropylamine and 27.0 grams (0.33 mole) pyridine. Analysis (percent): C, 73.15 (theory 74.99); H, 12.01 (theory 11.93); and N, 3.67 (theory 3.97) confirm the preparation.

#### Example 6

45 Methoxyethyleamide.—This material was prepared by the procedure of Example 1 from 100 grams (0.33 mole) of oleoyl chloride, 24.4 grams (0.33 mole) of methoxyethylamine and 27.0 grams (0.33 mole) pyridine. Analysis (percent): C, 73.08 (theory 74.55); H, 11.98 (theory 11.83); and N, 3.31 (theory 4.14) confirm the preparation.

#### Example 7

50 Oleoylmorpholine.—This material was prepared by the procedure of Example 1 from 100 grams (0.33 mole) of oleoyl chloride, 28.7 grams (0.33 mole) of morpholine and 27.0 grams (0.33 mole) of pyridine.

## Example 8

N,N-dibutyloleamide.—This product was prepared following the exact procedure of Example 2 except for the substitution of oleoyl chloride by linoleoyl chloride.

## Example 9

N,N-dibutyl-9,10-epithiostearamide.—120 grams (0.30 mole) of N,N-dibutyloleamide was epoxidized by the addition with stirring of 62.0 grams (0.36 mole) of meta-chloroperbenzoic acid in 630 ml. of chloroform. Reaction was continued for 1 hour beyond final addition and the excess peracid destroyed by a small amount of a 10% solution of  $\text{Na}_2\text{SO}_3$ . The metachlorobenzoic acid was removed by a  $\text{NaHCO}_3$  wash, followed by water washing. The  $\text{CHCl}_3$  solution was then dried with anhydrous  $\text{Na}_2\text{SO}_4$  and the  $\text{CHCl}_3$  stripped off to recover the product N,N - dibutyl-9,10-epoxystearamide, oxirane content 3.45% (theory 3.91%). 100 grams (0.24 mole) of this product was added to a well stirred slurry of 55.7 g. (0.73 mole) of thiourea and 89.5 g. (0.73 mole) of benzoic acid in acetone. Stirring was continued for 3 hours beyond the terminal addition whereupon the benzoic acid was washed out with 38.8 g. (0.36 mole) of  $\text{Na}_2\text{CO}_3$  and the organic product extracted with hexane. The organic phase extract was dried and stripped to recover the product N,N-dibutyl-9,10-epithiostearamide containing 6.41% sulfur (theory 6.67%).

## Example 10

N - (9,10 - epithiostearoyl)morpholine.—This product was prepared by the exact procedure described in Example 9 except for the substitution of oleylmorpholine for the N,N-dibutyloleamide of Example 9. Analysis of product showed (percent): C, 71.22 (theory 69.34); H, 11.22 (theory 10.77); N, 3.66 (theory 3.68); S, 3.44 (theory 7.80).

## Example 11

N,N - dibutyl-9,10,12,13 - diepithiostearamide.—This product was prepared following the procedure described in Example 9 except for the replacement of the N,N-dibutyloleamide of Example 9 by N,N-dibutyllinoleamide, and a doubling of the molar ratios of all reagents. The product analyzed as follows (percent): C, 69.64 (theory 68.57); H, 10.93 (theory 10.76); N, 3.10 (theory 3.07); S, 11.7 (theory 14.06).

## Example 12

N-ethoxyethoxyethoxypropyl-9,10-epithiostearamide.—To 166 g. of N-ethoxyethoxyethoxypropyl oleamide, Example 3, was added dropwise and with stirring 73.8 g. of m-chloroperbenzoic acid in 800 ml. of  $\text{CHCl}_3$ . The spent m-chloroperbenzoic acid was removed with 10% aqueous  $\text{NaHCO}_3$  and the epoxide recovered by drying and stripping off the  $\text{CHCl}_3$ . 171 g. of this epoxide was added dropwise to a slurry of 56 g. thiourea in 1000 ml. of acetone and the concurrent addition of 43.4 g. of glacial acetic acid and the reaction mixture stirred for 3 hours. The glacial acetic acid was neutralized with  $\text{Na}_2\text{CO}_3$  and the episulfide, N-ethoxyethoxyethoxypropyl-9,10-epithiostearamide, extracted with Skellysolve B and washed, dried, and stripped. Its elemental analysis was (percent): C, 67.1 (66.52); H, 11.42 (10.88); N, 2.67 (2.87); S, 2.29 (6.57).

## Example 13

N - ethoxyethoxyethoxypropyl - 9(10)mercaptostearamide.—173 g. of N-ethoxyethoxyethoxypropyloleamide in  $\text{CCl}_4$  was treated in the cold with a  $\text{CCl}_4$  solution containing 60.9 g. of bromine. Any unreacted bromine was removed by a thiosulfate wash. 140 g. of the resulting dibromo compound was added dropwise to a well stirred solution of 72 g. of  $\text{Na}_2\text{S} \cdot 9\text{H}_2\text{O}$  in dimethylsulfoxide maintained at 80° C. Stirring was continued at 80° C. for 3 hours. Water was added and the reaction product was

extracted with hexane; washed, dried, and stripped. Elemental analysis of the product was (percent): C, 66.3 (66.5); H, 11.1 (10.9); N, 2.7 (2.9); S, 4.4 (6.8).

## Example 14

5 N,N - dibutyl - 9(10) [dibutylphosphono]stearamide.—100 g. of N,N-dibutyloleamide, Example 2, 148 g. of dibutyl phosphite, and 1.29 of benzoyl peroxide catalyst were heated at 115° C. for 3½ hours. Additional units of 1.29 g. of benzoyl peroxide was added after the first and second hours of reaction time. The excess dibutyl phosphite was then removed by distillation at reduced pressure, 0.45 mm. Hg. The stillpot contents showed strong adsorption bonds at 8, 9.3, and 9.7 microns characteristics of the phosphonate group. The elemental analysis was (percent): C, obs. 71.46 (69.50); H, obs. 12.42 (11.92); N, obs. 2.20 (2.38); P, obs. 4.24 (5.28) respectively.

## Example 15

20 10 N-9,10-12,13-diepithiostearoylmorpholine.—This product was prepared by the same procedure described in Example 9 except for the substitution of linoleoyl morpholine for the N,N-dibutyloleamide of Example 8 and the doubling of molar proportions of the m-chloroperbenzoic acid in the epoxidation step and the thiourea and benzoic acid in the "epithioation" step. The elemental analysis was (percent): C, obs. 68.89 (63.92); H, obs. 10.26 (9.44); N, obs. 3.29 (3.38); S, obs. 4.00 (15.49) respectively.

## Example 16

30 35 40 45 N,N-dibutyl-[9(10)-hydroxy-(9)10-dibutylphosphato]stearamide.—44.7 g. of dibutylhydrogen phosphate was added to 182.2 g. of N,N-dibutyl-9,10-epoxystearamide at 90-95° C. with stirring. Reaction conditions were continued for 3½ hours after termination of the addition. The reaction product was dissolved in commercial hexane and the unreacted dibutyl hydrogen phosphate neutralized and washed out with portions of aqueous 10%  $\text{NaHCO}_3$  followed by several water washes. Acidulation of the hexane phase with diluted HCl followed by several water washes, drying and stripping, yielded the product. Elemental analysis was (percent): C, obs. 66.56 (65.91); H, obs. 11.04 (11.30); N, obs. 2.90 (2.26); P, obs. 3.04 (4.20).

## Example 17

50 55 N - [9(10)mercapto - (9)10-dibutylphosphatostearoyl]morpholine.—12 g. of dibutylhydrogen phosphate was added dropwise with stirring to 51.0 g. of (9,10-epithiostearoyl)morpholine, the preparation of Example 10, at 85-90° C. and the heating and stirring continued for 3 hours beyond the terminal addition. The reaction product was dissolved in commercial hexane and any excess or unreacted



60 65 was neutralized and washed out with aqueous 10%  $\text{NaHCO}_3$ . The hexane extract was washed several times with water dried and stripped. The elemental analysis of the product was (percent): C, obs. 66.74 (69.36); H, obs. 10.69 (11.05); N, obs. 2.89 (3.32); S, obs. 3.27 (2.17); P, obs. 1.68 (2.10) respectively.

## Example 18

The compounds prepared in accordance to the procedures given in Examples 1 through 7 were evaluated as base lubricants in the Shell Four-Ball Wear tests following a modified procedure of ASTM D2266-67. The resulting scar diameter on the balls after running at 600 r.p.m. for 1 hour at 120° C. and 50 kg. load were compared with the scars obtained using commercial lubricants such as Aeroshell Mil-L-708 (di-2-ethylhexyl sebacate

and additive), Gulfpride, single G, MS, multiviscosity, and 100 sec. paraffin oil. The results of these tests are reported in Table I.

TABLE I.—ANTIWEAR LUBRICANT PROPERTIES OF FATTY ACID AMIDES

| Compound                                                             | Avg. wear scar, mm. |                  |                                                                |
|----------------------------------------------------------------------|---------------------|------------------|----------------------------------------------------------------|
|                                                                      | With out additive   | With 5% additive | Additive                                                       |
| 1. N,N-bis(2-ethoxyethyl)oleamide.                                   | 0.597               | 0.735            | N,N-di-butyl-9,10-epithiostearamide.                           |
| 2. N,N-di-n-butyl-9,10-epithiostearamide.                            | 0.842               | -----            | None.                                                          |
| 3. Oleoylmorpholine.                                                 | 0.623               | 0.658            | Do.                                                            |
| 4. N,N-dimethyloleamide.                                             | 0.797               | 0.987            | Do.                                                            |
| 5. N,N-di-n-propyloleamide.                                          | 0.908               | 0.885            | Do.                                                            |
| 6. N,N-di-n-hexyloleamide.                                           | 0.893               | 0.898            | Do.                                                            |
| 7. N,N-di-n-butylsuccinamide.                                        | 0.758               | 0.798            | Do.                                                            |
| 8. N,N-di-n-butyl amide of sel. hydrogenated cottonseed fatty acids. | 0.798               | 0.958            | Do.                                                            |
| 9. N,N-bis(2-methoxyethyl)oleamide.                                  | 0.626               | 0.725            | Do.                                                            |
| 10. N,N-dibutyloleamide.                                             | 0.710               | -----            |                                                                |
| 11. N-oleoyl-4-propylpiperidine.                                     | 0.847               | -----            |                                                                |
| 12. Morpholide of sel. hydrogenated cottonseed fatty acids.          | 0.642               | -----            |                                                                |
| 13. N-methyl-N-butyloleamide.                                        | 0.607               | -----            |                                                                |
| 14. N-ethoxyethoxyethoxypropyloleamide.                              | 0.503               | -----            |                                                                |
| 15. N-ethoxyethoxypropyloleamide.                                    | 0.526               | -----            |                                                                |
| 16. N-methoxysopropyloleamide.                                       | 0.705               | -----            |                                                                |
| 17. N-methoxyethyloleamide.                                          | 0.420               | -----            |                                                                |
| 18. 102 sec paraffin oil.                                            | -----               | 0.902            | N-methoxyethyloleamide.                                        |
| 19. D.O.S.                                                           | -----               | 0.906            | Do.                                                            |
| 20. N,N-di-butyl-9(10)-carbo-butoxyoctadecanamide.                   | 0.610               | -----            |                                                                |
| 21. 102 sec paraffin oil.                                            | -----               | 0.818            | N,N-di-butyl-9(10)-carbo-butoxyoctadecanamide.                 |
| 22. D.O.S.                                                           | -----               | 0.945            | Do.                                                            |
| 23. N-[9(10)-mercapto-(9)10-dibutylphosphatostearoyl]morpholine.     | 0.615               | -----            |                                                                |
| 24. 102 sec paraffin oil.                                            | -----               | 0.552            | N-[9(10)-mercapto-(9)10-dibutylphosphatostearoyl]morpholine.   |
| 25. D.O.S.                                                           | -----               | 0.535            | Do.                                                            |
| 26. N,N-di-butyl-[9(10)-hydroxy-(9)10-dibutylphosphato]stearamide.   | 0.498               | -----            |                                                                |
| 27. 102 sec paraffin oil.                                            | -----               | 0.498            | N,N-di-butyl-[9(10)-hydroxy-(9)10-dibutylphosphato]stearamide. |
| 28. D.O.S.                                                           | -----               | 0.498            | Do.                                                            |
| 29. N,N-di-butyl-9(10)-[dibutylphosphono]stearamide.                 | 0.530               | -----            |                                                                |
| 30. N-ethoxyethoxyethoxypropyl-9,10-epithiostearamide.               | 0.707               | -----            |                                                                |
| 31. N-ethoxyethoxyethoxypropyl-9(10)-mercapto-stearamide.            | 0.690               | -----            |                                                                |
| 32. N-(9,10-12,13-diepithio-stearoyl)morpholine.                     | 0.665               | -----            |                                                                |
| 33. Bis(2-ethylhexyl)sebacate.                                       | 0.872               | -----            |                                                                |
| 34. 100 sec paraffin oil.                                            | 0.803               | -----            |                                                                |
| 35. Aeroshell (Mil-7808).                                            | 0.557               | -----            |                                                                |
| 36. Gulfpride, Single G, MS, multiviscosity.                         | 0.447               | -----            |                                                                |
| 37. 100 sec paraffin oil.                                            | -----               | 0.813            | N,N-di-butyl-9,10-12,13-diepithiostearamide.                   |
| 38. Bis(2-ethylhexyl)sebacate.                                       | 0.836               | Do.              |                                                                |
| 39. 100 sec paraffin oil.                                            | -----               | 0.723            | N-9,10-epithiostearoyl morpholine.                             |
| 40. Bis(2-ethylhexyl)sebacate.                                       | 0.915               | Do.              |                                                                |
| 41. 100 sec paraffin oil.                                            | -----               | 0.917            | N,N-di-butyl-9,10-dichlorostearamide.                          |
| 42. Bis(2-ethylhexyl)sebacate.                                       | 0.848               | Do.              |                                                                |

It can be seen from the data presented that the N-alkoxyalkyl and N,N-di(alkoxyalkyl)oleamides, without the assistance of additives, exhibited wear characteristics (i.e., low scar diameters) comparable to the commercial controls Aeroshell and Gulfpride, which do contain additives to improve performance. N,N-di-butyl-[9(10)-hydroxy-(9)10-dibutylphosphato]stearamide and N-[9(10)-mercapto-(9)10-dibutylphosphatostearoyl]morpholine

not only exhibit low wear characteristics in themselves but also impart as additives such characteristics to paraffin oil and DOS base lubricants.

## Example 19

The various amides were evaluated as extreme pressure lubricants or additives in a Shell 4-ball extreme pressure tester at 1440 p.p.m. following ASTM Procedure D 2596-67T. Loads were increased in increments of 20 kg. to weld point and the test ran one minute or to weld whichever occurred first. Commercial hypoid fluid SAE #90 was employed as the control E.P. lubricant. The performance of the amides tested is given in Tables II, III, and IV.

15

TABLE II.—EXTREME PRESSURE TESTS (ASTM D2596-67T)

| Compound                                                        | Weld point  |            |            |
|-----------------------------------------------------------------|-------------|------------|------------|
|                                                                 | No additive | With 5% #2 | With 5% #2 |
| 1. N,N-bis(2-ethoxyethyl)oleamide.                              | 120         | 170        |            |
| 2. N,N-di-n-butyl-9,10-epithiostearamide.                       | 300         | -----      |            |
| 3. Oleoylmorpholine.                                            | 120         | 150        |            |
| 4. N,N-dimethyloleamide.                                        | 120         | 140        |            |
| 5. N,N-di-n-propyloleamide.                                     | 120         | 150        |            |
| 6. N,N-di-n-hexyloleamide.                                      | 120         | 180        |            |
| 7. N,N-di-n-butylsuccinamide.                                   | 120         | 200        |            |
| 8. N,N-di-n-butyl amide of hydrogenated cottonseed fatty acids. | 120         | 170        |            |
| 9. N,N-bis(2-methoxyethyl)oleamide.                             | 120         | 160        |            |
| 10. N-methyl-N-butyloleamide.                                   | 100         | -----      |            |
| 11. N,N-dibutyl-9,10-epithiostearamide.                         | 300         | -----      |            |
| 12. N,N-dibutyl-9,10-12,13-diepithiostearamide.                 | 440         | -----      |            |
| 13. N-ethoxyethoxyethoxypropyloleamide.                         | 120         | -----      |            |
| 14. N-ethoxyethoxypropyloleamide.                               | 120         | -----      |            |
| 15. N-methoxysopropyloleamide.                                  | 100         | -----      |            |
| 16. N-methoxyethyloleamide.                                     | 100         | -----      |            |
| 17. N-9,10-epithiostearoylmorpholine.                           | 380         | -----      |            |
| 18. Bis(2-ethylhexyl)sebacate.                                  | 120         | -----      |            |
| 19. 100 sec paraffin oil.                                       | 100         | -----      |            |
| 20. SAE #90 commercial hypoid fluid.                            | 280         | -----      |            |

40

TABLE III  
Evaluation of N,N-di-butyl-9,10-12,13-diepithiostearamide as an additive and as a base oil in extreme pressure tests. (ASTM D2596-67T)

| Base oil                                    | Percent additive | Load, kg. | Wear scar, mm.       |    |
|---------------------------------------------|------------------|-----------|----------------------|----|
|                                             |                  |           | 100 sec paraffin oil | Do |
| 100 sec paraffin oil                        | 5                | 140       | 1.90                 |    |
| Do                                          | 5                | 200       | 2.35                 |    |
| Do                                          | 5                | 220       | 2.75                 |    |
| Do                                          | 5                | 240       | 4 Weld               |    |
| Bis(2-ethylhexyl)sebacate                   | 5                | 120       | 1.51                 |    |
| Do                                          | 5                | 180       | 1.59                 |    |
| Do                                          | 5                | 190       | 2.47                 |    |
| Do                                          | 5                | 200       | 4 Weld               |    |
| Do                                          | 10               | 240       | 2.88                 |    |
| Do                                          | 10               | 260       | 3.55                 |    |
| Do                                          | 10               | 270       | 6 Weld               |    |
| N,N-di-butyl-9,10-12,13-diepithiostearamide | None             | 120       | 1.38                 |    |
| Do                                          | None             | 160       | 1.61                 |    |
| Do                                          | None             | 200       | 1.89                 |    |
| Do                                          | None             | 280       | 2.13                 |    |
| Do                                          | None             | 320       | 2.47                 |    |
| Do                                          | None             | 360       | 2.70                 |    |
| Do                                          | None             | 400       | 2.88                 |    |
| Do                                          | None             | 440       | 7 Weld               |    |

60

Extreme pressure tests on N-ethoxyethoxyethoxypropyl-9,10-epithiostearamide (PC-O-No. 7682)

| Base oil             | Additive  | Applied load, kg. | Avg. scar, mm. |    |
|----------------------|-----------|-------------------|----------------|----|
|                      |           |                   | 7682           | Do |
| 7682                 | None      | 120               | 1.05           |    |
| 7682                 | None      | 160               | 1.75           |    |
| 7682                 | None      | 240               | 2.35           |    |
| 7682                 | None      | 300               | 2.19           |    |
| 7682                 | None      | 340               | 2.55           |    |
| 7682                 | None      | 360               | 2.62           |    |
| 7682                 | None      | 380               | Weld           |    |
| 102 sec paraffin oil | 7682 (5%) | 120               | 2.28           |    |
| Do                   | 7682 (5%) | 140               | 2.46           |    |
| Do                   | 7682 (5%) | 150               | Weld           |    |
| D.O.S.               | 7682 (5%) | 120               | 2.23           |    |
| D.O.S.               | 7682 (5%) | 140               | 2.44           |    |
| D.O.S.               | 7682 (5%) | 150               | Weld           |    |

75

See footnotes at end of table.

TABLE III—Continued

| Base oil                                                                                                | Additive  | Applied load, kg. | Avg. scar, mm.    |
|---------------------------------------------------------------------------------------------------------|-----------|-------------------|-------------------|
| Extreme pressure tests on N-ethoxyethoxyethoxypropyl-9(10)-mercapto-stearamide (PC-O-No. 7683)          |           |                   |                   |
| 7683                                                                                                    | None      | 200               | 1.54              |
| 7683                                                                                                    | None      | 300               | 2.26              |
| 7683                                                                                                    | None      | 400               | 2.25              |
| 7683                                                                                                    | None      | 450               | 2.15              |
| 7683                                                                                                    | None      | 500               | <sup>2</sup> 2.15 |
| 102 sec paraffin oil                                                                                    | 7683 (5%) | 120               | 1.97              |
| Do                                                                                                      | 7683 (5%) | 140               | 2.35              |
| Do                                                                                                      | 7683 (5%) | 150               | 2.54              |
| Do                                                                                                      | 7683 (5%) | 160               | Weld              |
| D.O.S                                                                                                   | 7683 (5%) | 120               | 1.68              |
| D.O.S                                                                                                   | 7683 (5%) | 140               | 2.18              |
| D.O.S                                                                                                   | 7683 (5%) | 160               | 2.59              |
| D.O.S                                                                                                   | 7683 (5%) | 170               | 2.72              |
| D.O.S                                                                                                   | 7683 (5%) | 180               | Weld              |
| Extreme pressure tests on N-(9,10-12,13-diepithiostearoyl)morpholine (PC-O-No. 7684)                    |           |                   |                   |
| 7684                                                                                                    | None      | 200               | 2.21              |
| 7684                                                                                                    | None      | 260               | 2.38              |
| 7684                                                                                                    | None      | 340               | 2.43              |
| 7684                                                                                                    | None      | 400               | 2.75              |
| 7684                                                                                                    | None      | 460               | 2.90              |
| 7684                                                                                                    | None      | 500               | <sup>2</sup> 2.98 |
| 102 sec paraffin oil                                                                                    | 7684 (5%) | 100               | 2.23              |
| Do                                                                                                      | 7684 (5%) | 120               | 2.61              |
| Do                                                                                                      | 7684 (5%) | 130               | 2.74              |
| Do                                                                                                      | 7684 (5%) | 140               | Weld              |
| D.O.S                                                                                                   | 7684 (5%) | 120               | 2.54              |
| D.O.S                                                                                                   | 7684 (5%) | 140               | 2.58              |
| D.O.S                                                                                                   | 7684 (5%) | 150               | Weld              |
| N-methoxyethyloleamide                                                                                  | 7684 (5%) | 140               | 2.53              |
| Do                                                                                                      | 7684 (5%) | 160               | 2.77              |
| Do                                                                                                      | 7684 (5%) | 170               | Weld              |
| Extreme pressure tests on N,N-dibutyl-9(10)-(dibutylphosphono) stearamide (PC-O-No. 7685)               |           |                   |                   |
| 7685                                                                                                    | None      | 120               | 3.05              |
| 7685                                                                                                    | None      | 140               | 4.50              |
| 7685                                                                                                    | None      | 150               | Weld              |
| Extreme pressure tests on N,N-dibutyl-[9(10)-hydroxy-9(10)-dibutyl-phosphato]stearamide (PC-O-No. 7686) |           |                   |                   |
| 7686                                                                                                    | None      | 200               | 0.887             |
| 7686                                                                                                    | None      | 300               | 2.78              |
| 7686                                                                                                    | None      | 340               | 4.32              |
| 7686                                                                                                    | None      | 350               | 4.50              |
| 7686                                                                                                    | None      | 360               | Weld              |
| 100 sec. paraffin oil                                                                                   | 7686 (5%) | 120               | 2.28              |
| Do                                                                                                      | 7686 (5%) | 140               | 2.80              |
| Do                                                                                                      | 7686 (5%) | 150               | 30.1              |
| Do                                                                                                      | 7686 (5%) | 160               | Weld              |
| D.O.S                                                                                                   | 7686 (5%) | 120               | 1.95              |
| D.O.S                                                                                                   | 7686 (5%) | 140               | 2.85              |
| D.O.S                                                                                                   | 7686 (5%) | 150               | 3.03              |
| D.O.S                                                                                                   | 7686 (5%) | 160               | Weld              |

40 We claim:

1. The compound N,N-dibutyl-9(10)-[dibutylphosphono]stearamide useful as a lubricant base.

## References Cited

## UNITED STATES PATENTS

|           |         |               |         |
|-----------|---------|---------------|---------|
| 3,189,628 | 6/1965  | Knight et al. | 260—403 |
| 3,211,766 | 10/1965 | Magne et al.  | 260—403 |
| 3,538,123 | 11/1970 | Mod et al.    | 260—403 |

50 ELBERT L. ROBERTS, Primary Examiner

8 TABLE III—Continued

Extreme pressure tests on N-[9(10)-mercapto-9(10)-dibutylphosphato]stearoylmorpholine (PC-O-No. 7687)

|        |      |     |                   |
|--------|------|-----|-------------------|
| 7687   | None | 120 | 0.608             |
| 7687   | None | 160 | 1.45              |
| 5 7687 | None | 200 | 1.40              |
| 7687   | None | 240 | 1.70              |
| 7687   | None | 280 | <sup>3</sup> 3.36 |

Extreme pressure tests on N,N-dibutyl-9(10)-carbobutoxyoctadecan amide (PC-O-No. 7688)

|      |      |     |      |
|------|------|-----|------|
| 7688 | None | 80  | 1.92 |
| 7688 | None | 90  | 2.18 |
| 7688 | None | 100 | 2.45 |
| 7688 | None | 120 | Weld |

<sup>1</sup> Incipient seizure.<sup>2</sup> Test stopped because of extreme decomposition. Did not weld.<sup>3</sup> Test stopped because of extreme decomposition and noxious fumes.

15 Did not weld.

<sup>4</sup> 5 seconds.<sup>5</sup> 4 seconds.<sup>6</sup> 10 seconds.<sup>7</sup> 46 seconds.

## 20 TABLE IV

Evaluation of N-9,10-epithiostearoyl morpholine as an additive and as a base oil in extreme pressure tests (ASTM D 2596-67T)

| Base oil                         | Percent additive | Load, kg. | Wear scar, mm.    |
|----------------------------------|------------------|-----------|-------------------|
| 25 100 sec. paraffin oil         | 5                | 120       | 2.00              |
| Do                               | 5                | 140       | 2.80              |
| Do                               | 5                | 160       | 3.25              |
| Do                               | 5                | 180       | <sup>1</sup> Weld |
| Bis(2-ethylhexyl)sebacate        | 5                | 80        | 1.57              |
| Do                               | 5                | 120       | 2.03              |
| Do                               | 5                | 140       | 2.41              |
| Do                               | 5                | 160       | 2.94              |
| Do                               | 5                | 180       | 3.00              |
| Do                               | 5                | 200       | <sup>2</sup> Weld |
| N-9,10-epithiostearoylmorpholine | None             | 120       | 0.70              |
| Do                               | None             | 200       | 2.13              |
| Do                               | None             | 240       | 2.43              |
| Do                               | None             | 300       | 2.68              |
| Do                               | None             | 380       | <sup>3</sup> Weld |

<sup>1</sup> 10 seconds. <sup>2</sup> 5 seconds. <sup>3</sup> 50 seconds.

45 We claim:

1. The compound N,N-dibutyl-9(10)-[dibutylphosphono]stearamide useful as a lubricant base.